

D. S. DE LAVAUD,  
HEAT TREATMENT FOR CENTRIFUGALLY CAST PIPES,  
APPLICATION FILED JULY 30, 1917.

1,280,418.

Patented Oct. 1, 1918.  
2 SHEETS—SHEET 1.

Fig. 1.



INVENTOR

Dimitri Sensaud de Lavaud

BY  
John Hallard Alcott  
his ATTORNEY

D. S. DE LAVAUD,  
HEAT TREATMENT FOR CENTRIFUGALLY CAST PIPES,  
APPLICATION FILED JULY 30, 1917.

1,280,418.

Patented Oct. 1, 1918.  
2 SHEETS—SHEET 2.



Dimitri Sénoud de Lavaud

BY

INVENTOR:

*John Wallace*  
ATTORNEY

# UNITED STATES PATENT OFFICE.

DIMITRI SENSAUD DE LAVAUD, OF NEW YORK, N. Y.

## HEAT TREATMENT FOR CENTRIFUGALLY-CAST PIPES.

1,280,418.

Specification of Letters Patent.

Patented Oct. 1, 1918.

Application filed July 30, 1917. Serial No. 183,503.

*To all whom it may concern:*

Be it known that I, DIMITRI SENSAUD DE LAVAUD, a citizen of the United States of Brazil, residing at 601 West 144th street, New York city, New York, U. S. A., have invented new and useful Improvements in Heat Treatment for Centrifugally-Cast Pipes, of which the following is a specification.

10 The present invention relates to the production of pipes of iron, steel or other metal cast under the influence of centrifugal force.

15 The object of the invention is to provide an improved heat treatment for centrifugally cast pipes or similar articles, whereby the speed of manufacture of the pipe is increased, and, this latter being the most important object, the quality of the pipes is bettered to a remarkable degree.

20 In particular, the prime object of the present invention is to produce a cast iron pipe which has a very fine grain, and in which the graphite exists in fine particles and not in coarse flakes as the case is with ordinary cast 25 iron pipes. This I accomplish by the following steps. First, the molten metal of which the pipe is to be formed is subjected to the action of centrifugal force, and at the same time rapidly cooled, the metal being preferably cooled within three to six seconds 30 after it has been poured into the mold. The casting, now of a white cast iron, is withdrawn from the mold immediately after solidification, the casting leaving the mold 35 at substantially 1500° Fahrenheit. The pipe is then superheated by elevating its temperature to from 1800° to 2000° Fahrenheit depending on the composition of the metal. The pipe metal changes over into 40 gray cast iron with graphite in fine particles, and any brittleness that may have been caused by the sudden cooling is removed. By this process a pipe of exceptionally fine 45 grained structure, strength and toughness is produced at a comparatively rapid rate.

The invention will be more clearly understood from the following description when taken in connection with the accompanying drawings illustrating an apparatus by which 50 the process of the present invention may be advantageously carried out, and a typical molecular structure of the gray cast iron product resulting from the process.

In these drawings,

55 Figure 1 shows the apparatus somewhat

diagrammatically and partially in section; and

Figs. 2, 3 and 4 are pen and ink replicas of microphotographs (450 diameters) of cross sections through a pipe, taken respectively 60 near the outside of the pipe, near the center and near the inside.

Referring to Fig. 1, 1 is a centrifugal casting machine from which a pipe 2 has been drawn by the supporting carriage 3. The 65 mold of this machine is preferably cooled by admitting water through the pipe 18. Means are provided for transferring the pipe to a superheating oven, which may be the crane 4, suitably supported in any manner as from 70 the I-beam 5. The oven may advantageously have a sloping floor 6 resting on suitable supports 8. The oven is provided with a roof 7, preferably of refractory material spaced suitably from the floor to allow of 75 the passage of the pipes therebetween. This roof may have an arched portion 9 where the heating is done, which may be by the admission of combustible gases through the apertures 10 when they are burned within the 80 oven. The oven is also provided with a stack 11 which may be fitted with a damper 12 for the regulation of the draft. The stack 11 is preferably placed so that the gases of combustion travel through the oven in the 85 same direction as the pipes.

After the pipes have been superheated they may be subjected to a coat of tar, and this is accomplished in the form of apparatus illustrated by providing at a suitable distance from the oven to allow of the pipes cooling to the proper temperature, a pit 13 containing tar 14. The tar may be kept in liquid condition by burning fuel on the grate 17. A baffle or guide 15 is provided for the 90 control of the passage of the pipes through the tar pit, and the pipes as they emerge are received on the platform 16.

The operation of the apparatus shown, 95 mechanically, is briefly as follows:

Molten metal is poured into the casting machine and the pipe cast and withdrawn from the machine in the usual manner. The pipe is then raised by the crane 4, revolved through a right angle, and deposited upon the upper end of the floor 6, whence it travels by its own weight slowly down the incline through the oven, being subjected to the heat of the burning gases emerging from the apertures 10. On emerging from the oven, 110

- the pipes enter the tar pit 13 and are guided therethrough by the baffle 15, the weight of the oncoming pipes being sufficient to cause the pipes to move through and out of the pit.
- 5 Thermally considered, the operation of the apparatus used in carrying out the process, is as follows:
- The metal in the centrifugal casting machine 1 which is being formed into a pipe 10 2 is rapidly cooled, as by water circulation through the pipe 18; the casting being formed and cooled within three to six seconds after the metal has been poured into the machine 1. The manner and rate of 15 cooling is such that when the casting is withdrawn from the mold, immediately after solidification, the casting is at the temperature of 1500° Fahrenheit. The pipe 2 is withdrawn from the machine by the 20 traveling carriage 3, engaged by the crane 4, and deposited at the right-hand end of the sloping floor 6 of the oven, and passes under the roof 7 and into the zone of the burners 10, with such celerity, preferably, 25 that the superheating treatment of the pipe commences very soon after the pipe is withdrawn from the mold, that is, before the pipe cools by contact with the atmosphere to a temperature appreciably lower than 1500° 30 Fahrenheit. During the passage of the pipe through the oven the temperature of the pipe is elevated from 1800° to 2000° Fahrenheit, depending on the composition of the metal.
- 35 The process of the present invention will perhaps better be understood if it is explained that iron cast in sand molds cools very slowly, ordinarily, its latent heat diffusing gradually. The iron being a liquid, 40 it crystallizes as it approaches the solid state, and the essential ingredients or impurities, so to speak, separate out and become entrapped or inclosed in the finally solid mass.
- 45 The principal constituent or impurity in cast iron is the carbon which exists in the graphitic state—really pure carbon which separates out as the iron cools. It usually exists in flakes or plates, often large—always so if the iron cools slowly. But whether the iron cools slowly or rapidly, these flakes or plates, that is, the lamella structure familiar to metallurgists, persists, at least to a deleterious extent. The carbon 50 in slowly cooled iron is found in larger globules or flakes than in iron that cools more quickly. Thus, iron cast in a permanent metal mold, whether it revolves or not, contains smaller crystals of carbon as well as of all other constituents. And when the iron, so cooled, is removed at once into the air, the cooling or accelerated formation of the crystals is accentuated. So that one of the features of the present invention, or rather one of the steps of the preferred
- process, is to cool the metal rapidly as it is being formed into the casting in the centrifugal casting machine, so that the pipe is formed and the casting cooled within three to six seconds after the metal is poured into 70 the rotating mold of the machine. The real essence of the present invention, however, is my discovery, further, that when the casting is solidified in the mold, rapidly cooled in the mold, and rapidly extracted from the 75 mold, preferably at the instant of solidification and when the casting is substantially at 1500° Fahrenheit, the quality of the casting may be improved to a remarkable extent, as compared with any heat treatment heretofore suggested, if the casting is superheated by elevating its temperature to from 1800° to 2000° Fahrenheit depending on the composition of the metal. These latter temperatures are largely empirical, as is also the 80 1500°, and are therefore not intended to be here stated in a limiting way, but merely as illustrative of what actual experiment with various different compositions of metals have shown me. With most if not all of these 85 compositions of metals, the 1500° temperature has been found so far to be ideal at the instant of extraction of the casting from the mold; but in the case of the superheating temperature, this has varied, so far as noted 90 between 1800° and 1980° Fahrenheit as the ideal superheating temperature, depending on the composition of the metal.
- When the pipe is withdrawn, at the 1500° temperature, it has a chilled outer surface. 100 In certain cases, of special mixtures, the pipe is chilled throughout. It cannot be filed or drilled by tool steel, and cannot in fact be worked by any instrument whatever. The chill consists of cementite and 105 pearlite, with a few black spots showing graphite. A layer of pure pearlite may be formed at the surface. The crystals are of needle formation. Near the center of the casting, that is, toward the inner wall of 110 the pipe, white dendrites of silico-ferrite are found, surrounded by a mass of fine graphite and ferrite. Sometimes the pearlite, distinctly lamella, may be seen, with cementite-phosphid eutectic.
- 115 After the pipe has been molded in a centrifugal machine, withdrawn from the mold, and superheated according to the present invention, however, the grain will be entirely normal and regular, and the casting will be very “close”-grained, that is to say, the grain will be very small. The pipe metal is soft and may be easily machined. As 120 illustrated in Figs. 2, 3 and 4, the graphite is very fine on the outside and inside surfaces, but a little coarser at the center. The absence of coarse graphite plates is noticeable; very marked. The structure is to a certain extent similar to that of a sand casting, but there is much less pearlite. There 125 130

are white grains and dendrites of silico-ferrite and fine graphite and ferrite in the matrix of pearlite.

I claim:

- 5 1. A process for providing improved iron annulus-type castings, which consists in providing a metal rotary mold, feeding a charge of molten metal thereto and rotating the mold to compress the molten metal against 50  
10 the metal mold by centrifugal force, while congealing the molten metal within six seconds after pouring the metal into the mold, extracting the casting thereby formed from the mold after said congealing of the molten 55  
15 metal as quickly as the machine permits, and afterward subjecting the extracted casting to a temperature of at least 1800° Fahrenheit, and then permitting the thus superheated casting to cool.
- 20 2. A process for providing improved iron castings of the annulus-type, which consists in providing a metal rotary mold, feeding a charge of molten metal thereto and rotating the mold to compress the molten 60  
25 metal against the metal mold by centrifugal force, while congealing the molten metal within six seconds after pouring the metal into the mold, extracting the casting thereby formed from the mold in time to prevent 65  
30 the casting from losing in the mold more heat than the heat which the metal mold absorbs for the congealing, and afterward subjecting the extracted casting to a temperature of at least 1800° Fahrenheit, and  
35 then permitting the thus superheated casting to cool.

3. A process for providing improved iron castings of the annulus-type, which consists in providing a metal rotary mold, feeding a charge of molten metal thereto and rotating the mold to compress the molten metal against the metal mold by centrifugal force, while congealing the molten metal within six seconds after pouring the metal into the mold, extracting the casting thereby formed from the mold at the instant 70  
40 when the temperature of the casting is substantially 1500° Fahrenheit, then rapidly heating the extracted casting to a tempera- 75  
45

ture substantially between 1800° and 2000° Fahrenheit, depending on the composition of the metal, and then permitting the casting to cool.

4. A process for providing improved annulus-type iron castings, which consists in 55  
feeding a charge of molten metal to a metal rotary mold and rotating the mold to compress the molten metal against the metal mold by centrifugal force, while congealing the molten metal within six seconds after 60  
pouring the metal into the mold, extracting the casting thereby formed from the mold after said congealing of the molten metal as quickly as the machine permits, and afterward subjecting the extracted casting to a 65  
temperature of at least substantially 500° Fahrenheit less than the fusion temperature of the molten metal employed, and then permitting the casting to cool.

5. A casting of gray cast-iron of the annulus-type, having a structure very much similar to that of a sand casting, but with very much less pearlite; the grain being entirely normal and regular but the grain being very "close", that is to say, very small; 70  
75 the absence of coarse plates of graphite being noticeable, in fact very marked, with the graphite very fine on the outside and inside surfaces, but a little coarser at the center; the casting being soft and easily machined in all parts; there being present white grains and dendrites of silico-ferrite and grains of fine graphite and ferrite in a matrix of pearlite.

6. An iron casting of the annulus type 80  
85 having a molecular structure characterized by the fact that the graphite is very fine on the outside of the casting and increases in coarseness a little from the outside toward the center of the casting but in such manner that the outside of the casting may be easily worked by any tool; there being present dendrites and grains of silico-ferrite and grains of ferrite containing fine graphite surrounded by a net work of pearlite.

In testimony whereof I have signed my name to this specification.

DIMITRI SENSAUD DE LAVAUD.